

## 1

3,291,624

ACETYLATED DERIVATIVES OF DIALDEHYDES  
AND OF THEIR HEMIACETALS AS GELATIN  
HARDENERS

Roy Arthur Jeffreys, Harrow, and Donald M. Burness, 5  
Wealdstone, Middlesex, England, assignors to Eastman  
Kodak Company, Rochester, N.Y., a corporation of  
New Jersey  
No Drawing. Filed Aug. 21, 1963, Ser. No. 303,664  
5 Claims. (Cl. 106—125)

This invention relates to gelatin compositions containing therein as a hardener a diacyloxy compound of a certain type.

Various compounds have been suggested as gelatin hardeners. Some of these compounds have exhibited properties of one kind or another which limited their use in certain situations. For instance, formaldehyde has shown desensitizing characteristics in contact with certain highly sensitized photographic emulsions. Other hardeners have been so effective that thickening of gelatin coating compositions occurs very shortly after the hardener addition, hence, the urgency of almost immediate coating. Some hardeners have had toxic effects and have been avoided where possible in manufacturing operations. Other hardeners have shown tendencies to fog and stain photographic elements with passage of time.

One object of our invention is to provide compositions which will give hardened gelatin layers but which do not exhibit thickening upon incorporating the hardener in the coating composition. Another object of our invention is to provide hardeners for gelatin-silver halide photographic emulsions which do not adversely affect their sensitivity and do not fog or stain the emulsions. A further object of our invention is to provide gelatin coating compositions which provide layers which retain a high degree of flexibility upon storage or aging. Other objects of our invention will appear herein.

We have found that certain diacyloxy compounds added to gelatin compositions exert a hardening effect upon gelatin layers formed therefrom, particularly upon aging or the like of those layers. Almost any amount of these hardeners will exert hardening on the gelatin but to obtain a substantial hardening advantage it is desirable that at least 0.1% and preferably 5-5%, based on the weight of the gelatin, be incorporated in the gelatin coating composition.

The hardeners in accordance with our invention are represented by the following type formulas in which acetyl is used as the acyl group. If desired, other acyl groups may be employed but the acetoxy compounds are preferred having been found to be quite convenient for use as hardeners:



in which R is an alkyl of 1-4 carbon atoms and n equals 0-5.



## 2



The gelatin compositions such as photographic gelatin-silver halide photographic emulsions containing a hardener in accordance with the invention may be coated out onto a support such as paper, film base or the like, to form photographic elements.

The following examples illustrate the preparation of some hardeners useful in hardening gelatin in accordance with our invention.

## Example 1

Mixed 1,1,2,2-diacetoxydiethoxyethane isomers were prepared by refluxing a mixture of 1,1,2,2-tetraethoxyethane and acetic anhydride plus a drop of methylsulphate as the catalyst. See the article by Fiesselmann and Horndler, *Chem. Ber.*, 87, 911, (1954).

## Example 2

Twenty-two ml. of 1,1,3,3-tetraethoxypropane was mixed with 20 ml. of acetic anhydride and one drop of methylsulphate was added thereto. The mixture was refluxed overnight. The product was then distilled yielding mixed 1,1,3,3-diacetoxydiethoxypropane isomers.

## Example 3

Thirty grams of 1,1,2,2-tetramethoxyethane was reacted with 42 ml. of acetic anhydride with one drop of methyl sulphate by the method described in the preceding example. The product obtained after distillation of the reaction mixture was fractionally crystallized from petroleum distillate (B.P., 60-80°) to give the isomers of 1,1,2,2-diacetoxydimethoxyethane, M.P. 77° and 51°, described by Fiesselmann and Horndler, *Chem. Ber.*, 87, 908, 911 (1954).

## Example 4

2,5-diacetoxy-2,5-dihydrofuran was prepared by the method described by Clauson-Kaas, U.S. Patent No. 2,514,026.

## Example 5

2,3-diacetoxy-1,4-dioxane was prepared by the method of Boeseken, Tellegen and Henriquez, *J. Amer. Chem. Soc.*, 55, 1284, (1933).

The above hardeners were added to portions of a fine grain negative gelatino-silver bromoiodide emulsion in the proportions specified, the properties obtained being indicated in the following table. The emulsion originally contained 6-7% gelatin and the final emulsion pH was as designated.

| Final emulsion pH 8.4                                    | (a)  |       |            | (b)            |                |
|----------------------------------------------------------|------|-------|------------|----------------|----------------|
|                                                          | Fog  | Cont. | Rel. Speed | M.P.<br>(° F.) | M.P.<br>(° F.) |
| Control                                                  | 0.31 | 0.98  | 4.30       | 92             | 93             |
| Control+2,3-diacetoxyl-1,4-dioxan (0.3g./l.)             | 0.23 | 0.95  | 4.38       | 90             | 93             |
| Control+2,3-diacetoxyl-1,4-dioxan (1.0g./l.)             | 0.23 | 0.96  | 4.30       | 94             | 100            |
| Control+2,3-diacetoxyl-1,4-dioxan (3.0g./l.)             | 0.22 | 0.92  | 4.33       | 105            | 123            |
| Control+2,5-diacetoxyl-2,5-dihydrofuran (0.3g./l.)       | 0.25 | 0.98  | 4.30       | 92             | 155            |
| Control+2,5-diacetoxyl-2,5-dihydrofuran (1.0g./l.)       | 0.21 | 0.92  | 4.30       | 92             | >200           |
| Control+Example 1 product (0.3g./l.)                     | 0.34 | 0.98  | 4.20       | 93             | 190            |
| Control+Example 1 product (1.0g./l.)                     | 0.28 | 0.96  | 4.20       | 94             | 197            |
| Control+Example 1 product (3.0g./l.)                     | 0.24 | 0.94  | 4.20       | 94             | >200           |
| Control+diacetoxylmethoxy ethane (m.p. 77°) (0.3g./l.)   | 0.32 | 0.98  | 4.18       | 88             | 164            |
| Control+diacetoxylmethoxy ethane (m.p. 77°) (1.0g./l.)   | 0.27 | 0.94  | 4.23       | 90             | >200           |
| Control+diacetoxylmethoxy ethane (m.p. 77°) (3.0g./l.)   | 0.23 | 0.94  | 4.27       | 101            | >200           |
| Control+diacetoxylmethoxy ethane (m.p. 51°) (0.3g./l.)   | 0.27 | 0.98  | 4.28       | 90             | 180            |
| Control+diacetoxylmethoxy ethane (m.p. 51°) (1.0g./l.)   | 0.26 | 0.98  | 4.32       | 96             | >200           |
| Control+diacetoxylmethoxy ethane (m.p. 51°) (2.0g./l.)   | 0.24 | 0.99  | 4.26       | 96             | >200           |
| Control+diacetoxylmethoxy propane (Example 2) (0.3g./l.) | 0.29 | 0.98  | 4.20       | 96             | >200           |

(a) Tested 7 days after coating.

(b) Coatings tested after incubation at 42% R.H. and 120° F. for 2 weeks.

| Final emulsion pH 8.5                        | (c)  |            |                | 25 |  |
|----------------------------------------------|------|------------|----------------|----|--|
|                                              | Fog  | Rel. Speed | M.P.<br>(° F.) |    |  |
| Control                                      | 0.36 | 4.12       | 96             |    |  |
| Control+2,3-diacetoxyl-1,4-dioxan (0.3g./l.) | 0.30 | 4.21       | 100            |    |  |
| Control+2,3-diacetoxyl-1,4-dioxan (1.0g./l.) | 0.31 | 4.16       | 120            |    |  |
| Control+2,3-diacetoxyl-1,4-dioxan (3.0g./l.) | 0.34 | 4.05       | 160            |    |  |

(e) Coatings tested after 3 months.

| Final emulsion pH 8.4                                    | (a)  |       |            | (b)            |                |
|----------------------------------------------------------|------|-------|------------|----------------|----------------|
|                                                          | Fog  | Cont. | Rel. Speed | M.P.<br>(° F.) | M.P.<br>(° F.) |
| Control                                                  | 0.22 | 0.99  | 4.20       | 94             | 105            |
| Control+2,5-diacetoxyl-2,5-dihydrofuran (0.3g./l.)       | 0.20 | 0.97  | 4.22       | 96             | 155            |
| Control+2,5-diacetoxyl-2,5-dihydrofuran (1.0g./l.)       |      |       |            | 96             | >200           |
| Control+2,5-diacetoxyl-2,5-dihydrofuran (3.0g./l.)       | 0.17 | 0.93  | 4.21       | 96             | >200           |
| Control+diacetoxylmethoxy ethane (m.p. 77°) (0.3g./l.)   | 0.22 | 0.98  | 4.25       | 90             | 105            |
| Control+diacetoxylmethoxy ethane (m.p. 77°) (1.0g./l.)   | 0.20 | 1.02  | 4.24       | 90             | 130            |
| Control+diacetoxylmethoxy ethane (m.p. 77°) (3.0g./l.)   | 0.22 | 0.91  | 4.22       | 90             | 180            |
| Control+diacetoxylmethoxy propane (Example 2) (0.3g./l.) | 0.22 | 0.97  | 4.26       | 96             | >200           |

(a) Tested 7 days after coating.

(b) Coatings tested after incubation at 42% R.H. and 120° F. for 2 weeks.

| Six Month Keeping Test                       | Final Emulsion pH |            |                |        |            |                |
|----------------------------------------------|-------------------|------------|----------------|--------|------------|----------------|
|                                              | pH 6.5            |            |                | pH 8.5 |            |                |
|                                              | Fog               | Rel. Speed | M.P.<br>(° F.) | Fog    | Rel. Speed | M.P.<br>(° F.) |
| Control                                      | 0.25              | 4.32       | 130            | 0.38   | 4.26       | 150            |
| Control+2,3-diacetoxyl-1,4-dioxan (0.3g./l.) | 0.24              | 4.28       | 150            | 0.39   | 4.22       | 170            |
| Control+2,3-diacetoxyl-1,4-dioxan (1.0g./l.) | 0.25              | 4.28       | 155            | 0.32   | 4.16       | >200           |
| Control+2,3-diacetoxyl-1,4-dioxan (3.0g./l.) | 0.21              | 4.28       | 190            | 0.30   | 4.06       | >200           |

Melting points were determined by immersing the element containing the gelatin coating in water and increasing the temperature until disintegration of the coating occurred.

We claim:

1. A composition of matter composed of gelatin containing a hardener selected from the group consisting of



in which R is an alkyl of 1-4 carbon atoms and  $n=0-5$ ;



and



- 5      2. A composition of matter composed of gelatin containing as a hardener therein diacetoxymethoxyethane.

3. A composition of matter composed of gelatin containing as a hardener therein diacetoxymethoxypropane.

4. A composition of matter composed of gelatin containing as a hardener therein diacetoxymethane.

10     5. A composition of matter composed of gelatin containing as a hardener therein diacetoxymethoxyfuran.

### References Cited by the Examiner

UNITED STATES PATENTS

- |           |        |         |       |        |
|-----------|--------|---------|-------|--------|
| 2,585,596 | 2/1952 | Stanton | ----- | 96-111 |
| 2,870,013 | 1/1959 | Harrow  | ----- | 96-100 |
| 3,241,972 | 3/1966 | Wilson  | ----- | 96-111 |

MORRIS LIEBMAN *Primary Examiner*

D. J. ARNOLD, *Assistant Examiner.*

UNITED STATES PATENT OFFICE  
CERTIFICATE OF CORRECTION

Patent No. 3,291,624

December 13, 1966

Roy Arthur Jeffreys et al.

It is hereby certified that error appears in the above numbered patent requiring correction and that the said Letters Patent should read as corrected below.

Column 1, lines 53 to 57, for the right-hand portion of the formula reading

00OCH<sub>3</sub>      read      OCOCH<sub>3</sub>

same column 1, lines 60 to 63, the formula should appear as shown below instead of as in the patent:



column 2, lines 1 to 5, the formula should appear as shown below instead of as in the patent:



columns 3 and 4, in the heading to the third table, first column for "8.4" read -- 6.5 --.

Signed and sealed this 24th day of October 1967.

(SEAL)  
Attest:

EDWARD M. FLETCHER, JR.  
Attesting Officer

EDWARD J. BRENNER  
Commissioner of Patents